

April 18, 1933.

D. WESTAD

1,904,894

PROCESS AND APPARATUS FOR THE MANUFACTURE OF CELLULOSE

Filed April 4, 1931

3 Sheets-Sheet 1



Inventor:  
Daniel Westad

By  
Pennie Davis Marvin & Edmunds  
attorneys

April 18, 1933.

D. WESTAD

1,904,894

PROCESS AND APPARATUS FOR THE MANUFACTURE OF CELLULOSE

Filed April 4, 1931

3 Sheets-Sheet 2



Inventor:  
D. Westad;  
By  
Penrice, Davis, May & Edwards,  
The Attorneys

April 18, 1933.

D. WESTAD

1,904,894

PROCESS AND APPARATUS FOR THE MANUFACTURE OF CELLULOSE

Filed April 4, 1931

3 Sheets-Sheet 3

Fig. 4.



Fig. 5.



Inventor:  
D. Westad;  
By:  
Pearce, Davis, Quinn & Ward  
His Attorneys.

## UNITED STATES PATENT OFFICE

DANIEL WESTAD, OF BYGDOY NEAR OSLO, NORWAY

## PROCESS AND APPARATUS FOR THE MANUFACTURE OF CELLULOSE

Application filed April 4, 1931, Serial No. 527,672, and in Norway May 27, 1930.

This invention relates to the manufacture of cellulose by heating wood chips or other cellulosic materials under pressure with aqueous solutions of chemicals capable of dissolving the incrustations of the raw material, thus liberating the cellulose fibres, and the invention has for its object a method of carrying this process into effect, which allows of obtaining an increased yield of cellulose of 10 first class quality as compared with the processes hitherto employed.

It is a well known fact that the output of cellulose obtained under the present practice do not by far correspond to the percentage 15 of cellulose fibres contained in the raw materials (wood, straw etc.), a considerable proportion of the fibres being in fact lost during the digestion operation. This loss is to a 20 great extent due to the fact that the raw material is subjected to a very uneven attack of the dissolving chemicals, so that the fibres first liberated will become destroyed before the remainder of the charge has been sufficiently acted upon.

25 According to the present invention these drawbacks are avoided by combining the digestion operation at elevated temperatures with a preparatory treatment of the wood chips or other cellulosic raw material with 30 digestion liquor at low temperatures, but under high pressure.

This method of operation allows of a considerable shortening of the time, in which the material is subjected to high temperatures 35 and thus also an important decrease in the consumption of steam, at the same time as an increased output of first class cellulose is obtained.

The digestion operation and the preparatory treatment with digestion liquor at low 40 temperatures under high pressure may be carried out in the same vessel, viz. an ordinary digestor, but it is preferred to carry the operations into effect as separate steps in 45 two or more separate sets of containers, so arranged in relation to one another that the material (wood chips and the like) can be readily transferred from one set of containers to another.

50 As will be understood, the process accord-

ing to the invention is composed of two main phases: the impregnation phase and the digestion or cooking phase. During the impregnation stage, the cellulosic material (wood chips and the like) is subjected to the action of digestion liquor under a high pressure, but at a relatively low temperature (viz. below 100° C., usually between 70° and 15° C. and even down to near zero).

Prior to the impregnation with digestion liquid, when employed as a step in such digestion process which is carried out by the use of sulphite solutions—or other solutions prepared by the use of gaseous reaction components—may go a treatment of the chips 55 with the gaseous reagent or reagents. This treatment with gaseous reagents may also suitably be effected at low temperatures and in the same container as that in which the subsequent impregnation with liquid under pressure takes place. The gas may be applied under ordinary or increased pressure and even under pressures sufficiently high to bring about partial or complete condensation of the gas.

When the invention is applied to the soda- 75 or sulphate-process or to other processes, in which gaseous reaction components are ordinarily not made use of, the preparatory treatment which is referred to above, will be omitted, although it may under certain circumstances be considered desirable from particular reasons to combine even these types of processes with a preparatory treatment with some gaseous reagent.

In the preferred embodiment of the invention, the impregnation step and the digestion step are carried out in different vessels, and these vessels are suitably arranged above one another. Thus the impregnation vessel may be arranged on the floor above the digestors, so that the mixture of impregnated chips and 80 impregnation liquid can be transferred to the digestor under the action of its own weight. The transfer of the charge is facilitated by giving to the containers a form, adapted for 85 the purpose. The form of the vessel is suitably so elected as to promote as far as possible the utilization of the gravity of the charge to convert same into a cyclonic centripetal mo- 90 95 100

tion. It is suitable for the purpose in question to use containers, having tapering side walls, so that the sectional areas increase towards the bottom of the container. It is also 5 suitable to arrange the discharge opening so that its center lies outside of a vertical line through the center of gravity of the charge.

A suitable container may for example be 10 considered as composed of a conical main portion and a non-symmetrically cup-shaped bottom portion, having a deepened part, in which the discharge opening is placed eccentrically in relation to the container walls. Experience has proved that a vessel so constructed 15 can readily be emptied of a charge consisting of wood chips and liquid.

In order to promote the discharge of the material, it may also be of advantage to provide the bottom portion of the container 20 around the discharge opening with recesses, ribs or vanes, so arranged as to form an angle with radial lines through the center of the discharge opening. Otherwise any type of container may be used for the preparatory 25 treatment of the chips, provided that they allow of rapid and complete emptying of the contents. The vanes or ribs referred to above may with advantage be used in containers of any type and in combination with eccentrically as well as with centrally arranged discharge openings. It is no necessary condition 30 that the vanes are arranged immediately adjacent to the outlet or at the bottom of the container. The desired effect will be produced also when the vanes are arranged on or 35 near to the side walls of the container.

When containers without guide ribs or vanes, or containers with centrally arranged discharge outlet are made use of, it will usually 40 be necessary to arrange very large outlet channels or to make use of moving emptying members or agitators of one kind or another.

A plane for carrying the invention into effect may for example consist of two spherical 45 digestors of  $20 \text{ m}^3$  capacity each one preheating container of  $32 \text{ m}^3$  capacity above said digestors and two "interim tanks" (impregnation containers) with a capacity of each 46  $\text{m}^3$ , arranged above the said preheating 50 containers.

A plant of this type is diagrammatically illustrated in the accompanying drawings in which

Fig. 1 is a diagrammatic representation of 55 the plant;

Fig. 2 is a vertical sectional view, on an enlarged scale, of one of the impregnation tanks;

Fig. 3 is a horizontal sectional view of the 60 same tank on lines III—III of Fig. 2;

Fig. 4 is a side view of the tank, partly in section on line IV—IV of Fig. 2, and

Fig. 5 is a horizontal sectional view of an 65 impregnation tank having guide members on the bottom.

1 and 2 represent the impregnation tanks, 3 the preheating (or precooking) container and 4 and 5 the digestors.

When cellulose is to be manufactured from wood chips according to the sulphite process 70 by the use of the illustrated plant, one may for example operate as follows:

The "interim tanks" (impregnation tanks) 75 1 and 2 are charged with chips, containing for example 32 per cent of moisture. This moisture percentage may be the result of a preceding soaking of the chips, in water or some aqueous solution of chemicals, or it may be the original moisture of the wood, from 80 which the chips have been cut.

Sulphur dioxide gas is now introduced into tank 1 through an inlet at the bottom. The gas displaces the air contained in the charge of chips and is absorbed in the water contained in the chips. When the chips have 85 become saturated with sulphurous acid (for example after about 5 minutes), liquid is introduced into the tank.

The introduced liquid may be a calcium bisulphite solution, containing lime ( $\text{CaO}$ ) in 90 sufficient excess to result in a digestion liquid of the ordinarily employed composition, when the sulphur dioxide taken up in the chips has been absorbed in the liquid.

The tank is wholly filled with liquid. To 95 avoid the undesirable results of differences in the concentration or composition of the impregnation liquid at different places in the impregnation vessel, it may be found desirable, when the vessel has been charged with liquid, to maintain the liquid in circulation for a short period of time, for example by means of a pump inserted in a pipe line, connecting the top and bottom parts of the impregnation vessel.

The tank is thereupon placed under a pressure of about 6 atmospheres by liquid (or gas) pressure, while the temperature is maintained below  $70^\circ \text{C}$ , for example at about  $20^\circ \text{C}$ . After about 6 hours, the pressure is relieved and the mixture of chips and liquid is run into the preheating vessel 3. Efficient mixing of chips and liquor is promoted by the cyclonic motion of the charge during the transfer to the preheating vessel, and may be 110 further promoted by pumping liquor from the bottom of the preheating vessel into the interim tank at a point above the charge.

The temperature in the charge thus introduced into the preheating vessel is now for 115 example about  $20^\circ \text{C}$ . The charge is then heated to boiling temperature. After about 3 hours, the charge is introduced into one of the digestors. The transfer and the mixing of chips and liquor is promoted by circulation of liquor as described in connection with the transfer from interim tank to preheating vessel.

The digestion operation is carried out in 120 the usual manner. After about 6 hours, the 125

process is terminated and the digestors emptied.

In the meantime, a new charge of chips has been prepared in the interim tank 2 and preheater 3 and run into the second digestor 5. The impregnation of this second charge in interim tank 2 takes place during the same period of time as that, in which the first prepared charge is under treatment in digestor 4.

The operation of the plant is thereupon continued in the same way by the constant use of the interim tanks and the preheating vessel to prepare new charges for introduction into the digestors.

All steps or phases of the process thus take place synchronously, and in these synchronous operations, the process differs fundamentally from what takes place when the various phases all take place in one and the same vessel as is the case in known processes for the manufacture of cellulose.

The above described method of operation is only to be considered as an example, in that the various details in the process itself as well as in the apparatus employed may be varied within wide limits and modified according to circumstances, for example so as to make it possible without reducing the capacity of the plant to produce at choice different qualities of pulp, requiring a shortened or extended digestion period.

When operating as above described, any other type of digestion liquid than calcium bisulphite may of course be employed, such as for example sulphite solution, in which the base is magnesia, potash, soda or ammonia or mixtures of two or more of these bases, with or without auxiliary additions, such as for example salts of strong acids etc. The employed bases or auxiliary additions may also be added in part to the digestion liquor, before it is brought into the impregnation vessel; but they may also be used at least in part to prepare the chips or other cellulosic raw material previously to the introduction of the sulphurous acid gas into the charge.

As regards the employed digestors, these may be of any known or suitable type.

It will be understood that the process as described may be carried out also without the use of special preheating vessels 3. In this case the charge is directly transferred from the impregnation tanks 1, 2 to the digestors 4, 5. The number of digestors will then have to be increased with one for each two impregnation tanks. The volumes of the digestors will then have to be dimensioned as for the preheating vessel in the described example.

The invention is not limited to the use of two or three sets of containers, but covers the execution of the process in any number of stages carried into effect in succession in separate containers, because in fact the utiliza-

tion of the interior space of various containers will be more complete, the greater the number of containers through which the chips have to pass. With the increase in number of vessels operating in series will follow also an increase in the homogeneity or uniformity of the resulting cellulose pulp as well as in the yield calculated on the employed raw material.

I claim:

1. A process of recovering cellulose from raw materials, comprising subjecting a charge of the raw material to impregnation with a digestion-liquid under a pressure raised several atmospheres above normal and at a temperature considerably below 100° C. in a closed impregnation vessel for a period of several hours, thereupon transferring the entire charge including the contained digestion liquid into another vessel, and then heating the charge consisting of impregnated raw material and digestion liquid to digestion temperatures considerably above 100° C. for a period of time sufficient to effect complete dissolution of the incrustations on the material.

2. A process according to claim 1, in which the impregnation treatment is effected at a temperature below 70° C. and under a pressure of at least 5 atmospheres.

3. A process of recovering cellulose from raw materials, comprising taking a charge of material, impregnating same with a digestion-liquid in one container, and thereupon transferring the charge into another container for continued treatment with digestion liquid, said digestion liquid being circulated from the container receiving the charge into and through the container from which material is being discharged, the said circulation being continued for a sufficiently long period of time to obtain a liquid of uniform composition in the receiving container.

4. A process for the recovering of cellulose from raw materials, comprising subjecting a batch of the raw material to impregnation with digestion liquid in an impregnation chamber for a definite period of time, subjecting another batch of the material to the same kind of impregnation in another impregnation chamber for the same period of time as that of the first named batch, transferring the first named batch in its entirety from the impregnation chamber into a secondary treating chamber and retaining same in this chamber for a definite period of time, removing the treated charge from said secondary treating chamber, and immediately afterwards transferring the second impregnated batch in its entirety directly from the second impregnation chamber into the secondary treating chamber and retaining same therein for the same period of time as the removed batch.

5. A container for impregnating cellulose-

materials with aqueous solutions of chemicals prior to digestion-treatment thereof in another container, the bottom of said container having the form of a trough sloping towards a point near the wall of the container, a discharge outlet for impregnated material being arranged at said point, and a downwardly directed discharge tube.

6. A container for impregnating cellulose  
10 materials with aqueous solutions of chemicals as a separate step prior to digestion-treatment thereof, in another container, the container having an overhanging wall and the bottom of the container having an eccentrically arranged discharge opening near said overhanging container-wall, said opening being located at a point towards which the bottom slopes from all sides.

7. A container according to claim 5, in  
20 which there is provided interior guide members so arranged in relation to the flow of the charge during discharge through the opening in the bottom that they effect a whirling motion of the charge around a vertical  
25 axis.

8. A multiple-stage process for recovering cellulose from raw materials in which a charge of the material is impregnated with reactive liquid in one container and is subjected to a final digestion treatment in another container, the duration of the impregnation treatment in relation to the duration of the digestion treatment being shortened or lengthened by decreasing or increasing respectively the number of impregnation containers in cooperative operation with the digestion containers.

9. Process of recovering cellulose from raw materials comprising subjecting a charge  
40 of the raw material to the action of gaseous sulphurous acid so as to effect absorption of gaseous sulphurous acid in the moisture in the interior of the individual pieces of raw material, thereupon subjecting the so prepared charge to impregnation with sulphite digestion liquid under a pressure raised several atmospheres above normal and at a temperature considerably below 100° C. in a closed impregnation vessel for a period of  
45 several hours, and thereafter heating the charge consisting of impregnated raw material and acid sulphite digestion liquor to digestion temperatures considerably above 100° C. for a period of time sufficient to effect dissolution of the incrustations of the material.

In testimony whereof I have signed my name unto this specification.

DANIEL WESTAD.